

Jan. 26, 1932.

A. W. HAHN

1,842,400

CONCENTRATION OF MINERALS

Filed Feb. 1, 1929



ALBERT W. HAHN.

By His Attorney

Anthony Mine

## UNITED STATES PATENT OFFICE

ALBERT W. HAHN, OF SALT LAKE CITY, UTAH

## CONCENTRATION OF MINERALS

Application filed February 1, 1929. Serial No. 336,742.

The invention relates to the treatment of difficult ores where, in a flotation system, a middling product is made which is in itself difficult to handle by flotation and which also <sup>5</sup> renders the original material more difficult to handle if returned to the head of the flotation system.

By the present process the flotation system is so operated as to segregate the difficult middlings and remove them from the circuit.

The invention is particularly useful in the concentration of oxidized or partially oxidized ores. In certain ores, the silver-bearing minerals are in a form difficult to concentrate and recover by flotation and when high recoveries are obtained the grade of the concentrate is relatively low, as excessive amounts of barren gangue particles are floated <sup>15</sup> with the desired silver mineral. These silver minerals, difficult to float, when returned to the flotation circuit for re-treatment or when treated in separate flotation machines drop out of the flotation froth and <sup>20</sup> produce a tailings or middling product relatively very high in silver values and high in barren gangue particles.

I propose, therefore, to segregate and remove these silver minerals, refractory to flotation concentration, instead of following the usual flotation practice of returning the tailings from the cleaner and the middlings concentrate to the circuit. By removing the relatively high silver-bearing flotation middling product and treating it separately by flotation, I have found by tests on the basis of treating approximately 90 tons per day of mixed oxide and sulphide lead-silver siliceous ores that the number of flotation cells <sup>30</sup> necessary to obtain the same grade of final tailings is about 30 per cent less than when following the standard practice.

In the concentration of ores by froth flotation, particularly oxidized or partially oxidized ores, I propose therefore to take off the highly siliceous concentrate or middling containing the refractory mineral or minerals, particularly the silver minerals, to subject this concentrate to further treatment as by <sup>45</sup> separate flotation or table concentration and

to dispose of the products, concentrates and tailings, from this separate treatment in such ways as will yield the maximum profit according to the character of the product.

For instance, if the concentrate from this <sup>55</sup> separately treated product is high in lead it can be combined with a regular flotation lead concentrate. The tailings relatively high in silver and siliceous gangue material can be advantageously smelted at a copper <sup>60</sup> smelter in which this type of material is desirable.

The accompanying drawing is a diagram illustrating by way of example an application of the invention to the concentration of <sup>65</sup> mixed oxide-sulphide lead-silver ores.

Numbers 1 to 14 are successive cells of a main flotation unit. Supplementary flotation units are shown with three cells E, with four cells F and three cells H respectively. <sup>70</sup> The ore pulp enters the feed box of the principal flotation unit at A and passes through the cells 1 to 14 in succession until the tailings are taken off at B.

The sulphide concentrates are first taken <sup>75</sup> off from cells 1 to 3, cleaned in the supplementary cells E and the finished sulphide concentrate taken off therefrom; the tailings passing off at G being carried around by the line C to the head of the sulphide circuit, cell No. 1.

The oxide concentrates are taken off from cells 4 to 11 and cleaned in cells F from which the finished oxide concentrate is taken off. The tailings run off at I and are carried <sup>85</sup> around by the line D to the cell 4 which is the head of the oxide concentrate circuit.

The oxidized minerals are floated by adding to the cells sodium sulphide, amylixanthate and a frothing agent if necessary, in various quantities, and at each of the cells or in every other cell, depending on the nature of the ore; and at times, it may be necessary to add small amounts of sodium silicate. <sup>90</sup>

From the last section of the main unit, cells 12, 13 and 14, there is drawn off a middlings; that is, a concentrate of lower value than those taken off from the previous cells. <sup>95</sup> <sup>100</sup>

In the ores to which this invention is particularly directed such middlings are high in gangue and in silver. They are difficult to float and they are particularly objectionable in this respect in the original pulp.

The removal of the middlings is effected in substantially the same manner as above set forth for the removal of the oxide concentrates.

10 I have found that the values in the ore can be more economically recovered by segregating these middlings and treating them separately. I limit the middlings thus taken off as far as is practicable to the distinct

15 product which contains only negligible quantities of the more easily floatable minerals.

According to the diagram such middlings are separately concentrated in cells H, the 20 middling concentrate going to a lead smelter and the tailings at J to a copper smelter.

To illustrate the dropping out of the refractory silver mineral when an oxidized lead-silver flotation concentrate is subjected 25 to a flotation cleaning operation as in the cells F, I submit the following results obtained by laboratory tests and tonnage mill tests.

*Oxide concentrate cleaner tests*

30 HEADS

| Au ozs. | Ag ozs. | Pb % | Cu - % | Fe % | Insol. % |
|---------|---------|------|--------|------|----------|
| 35      | 24.2    | 43.6 | 4.5    | 30.8 |          |
|         | 18.0    | 35.2 | 6.5    | 32.1 |          |
|         | 20.0    | 42.4 | 5.4    | 25.4 |          |
|         | 17.2    | 45.8 | 6.0    | 24.0 |          |
|         | 19.2    | 39.2 | 6.0    | 30.4 |          |
|         | 23.8    | 42.0 | 10.7   | 27.8 |          |

40 CLEANER CONCENTRATES

| Au ozs. | Ag ozs. | Pb % | Cu % | Fe % | Insol. % |
|---------|---------|------|------|------|----------|
| 45      | 24.3    | 52.4 | 4.5  | 18.4 |          |
|         | 21.8    | 47.0 | 5.2  | 20.9 |          |
|         | 19.4    | 48.2 | 4.0  | 18.4 |          |
|         | 19.2    | 52.8 | 4.6  | 19.2 |          |
|         | 18.4    | 45.0 | 5.3  | 18.4 |          |
|         | 24.1    | 42.8 | 6.0  | 26.8 |          |

CLEANER TAILS

| Au ozs. | Ag ozs. | Pb % | Cu % | Fe % | Insol. % |
|---------|---------|------|------|------|----------|
| 55      | 28.0    | 16.4 | 7.3  | 54.2 |          |
|         | 25.1    | 29.2 | 7.2  | 40.2 |          |
|         | 26.0    | 25.1 | 6.0  | 44.9 |          |
|         | 18.0    | 27.3 | 6.2  | 33.2 |          |
|         | 29.2    | 34.4 | 6.1  | 37.8 |          |
|         | 24.7    | 10.3 | 8.6  | 61.4 |          |

The above table shows an increase in the 60 lead content by the concentration, but no substantial increase in the silver content. And the cleaner tails show in each case an increased percentage in silver; indicating that the silver minerals have dropped out of the 65 froth or at least have not been floated there-

with. I submit also the following table of similar tests on the oxide middlings which are passed through the cleaner H.

*Oxide middling cleaner tests*

HEADS

| Au ozs. | Ag ozs. | Pb % | Cu % | Fe % | Insol. % |    |
|---------|---------|------|------|------|----------|----|
| .044    | 22.2    | 17.7 | .13  | 10.9 | 51.2     | 75 |
| -----   | 21.4    | 11.3 | .28  | 10.9 | 57.7     |    |
| -----   | 21.6    | 11.3 | .31  | 11.0 | 57.8     |    |
| -----   | 21.3    | 10.8 | .30  | 10.9 | 57.6     |    |
| -----   | 21.1    | 11.2 | .28  | 11.2 | 57.3     |    |
| -----   | 21.5    | 11.5 | .31  | 11.3 | 57.5     |    |
| -----   | 19.1    | 6.9  | .33  | 11.1 | 64.1     |    |

CLEANER CONCENTRATES

| Au ozs. | Ag ozs. | Pb % | Cu % | Fe % | Insol. % |    |
|---------|---------|------|------|------|----------|----|
| .06     | 26.5    | 46.4 | .05  | 7.5  | 21.8     | 80 |
| -----   | 26.6    | 13.1 | .32  | 12.5 | 50.8     |    |
| -----   | 32.2    | 14.8 | .32  | 13.4 | 42.2     |    |
| -----   | 29.8    | 16.1 | .38  | 12.8 | 46.0     |    |
| -----   | 33.8    | 15.3 | .40  | 13.7 | 45.3     |    |
| -----   | 28.5    | 14.0 | .38  | 13.6 | 49.3     |    |
| -----   | 50.1    | 30.6 | .50  | 16.2 | 23.2     |    |

TAILS

| Au ozs. | Ag ozs. | Pb % | Cu % | Fe % | Insol. % |    |
|---------|---------|------|------|------|----------|----|
| .04     | 21.1    | 9.5  | .15  | 11.8 | 59.6     | 95 |
| -----   | 17.3    | 9.8  | .25  | 9.6  | 63.2     |    |
| -----   | 18.0    | 10.1 | .30  | 10.2 | 61.4     |    |
| -----   | 15.6    | 7.3  | .24  | 9.7  | 65.4     |    |
| -----   | 16.7    | 9.7  | .23  | 10.2 | 61.8     |    |
| -----   | 15.9    | 9.5  | .28  | 9.4  | 64.1     |    |
| -----   | 13.1    | 3.9  | .25  | 10.0 | 70.0     |    |

The middling being treated separately in this way, the concentration brings about a substantial increase in the silver and lead. The metallic content of the tails however is high enough to make them worth adding to the charge in a copper smelter.

The following tables will illustrate the differences between the old method in which high recoveries are obtained, but with a low grade of concentrate, and the present method by which though the recoveries are lower, the concentration is relatively high. The raw material was a mixture of ores from the Tintic Standard Mining Company and the North Lily Mining Company. The results of the standard method of flotation are shown in the following Table A.

Table A

|                   | % Weight | Assay   |      |      |        | Recoveries—Per cent |       |       |       |
|-------------------|----------|---------|------|------|--------|---------------------|-------|-------|-------|
|                   |          | Ag ozs. | Pb % | Fe % | Ins. % | Ag                  | Pb    | Fe    | Ins.  |
| Heads-----        | 100.0    | 24.4    | 23.0 | 7.9  | 44.4   | 100.0               | 100.0 | 100.0 | 100.0 |
| Concentrates----- | 64.5     | 32.7    | 34.9 | 9.8  | 20.6   | 92.7                | 99.0  | 80.5  | 37.3  |
| Tails-----        | 34.5     | 5.05    | 0.62 | 4.3  | 78.4   | 7.3                 | 1.0   | 19.5  | 62.7  |

With the same ore, treated so as to obtain a better ratio of concentration, the results were in accordance with Table B.

Table B

| 5                 | % Weight | Assay   |      |      |        | Recoveries—Per cent |       |       |       |
|-------------------|----------|---------|------|------|--------|---------------------|-------|-------|-------|
|                   |          | Ag ozs. | Pb % | Fe % | Ins. % | Ag                  | Pb    | Fe    | Ins.  |
| Heads.....        | 100.0    | 20.4    | 16.0 | —    | 56.8   | 100.0               | 100.0 | 100.0 | 100.0 |
| Concentrates..... | 37.0     | 43.8    | 38.9 | 0.4  | 23.3   | 78.5                | 89.9  | —     | 15.2  |
| Tails.....        | 63.0     | 6.98    | 2.57 | —    | 56.8   | 21.5                | 10.1  | —     | 84.8  |

10 The higher recoveries are shown in Table A where, for example, the concentrates weigh 64.5 per cent compared with 37 per cent in Table B; and where the recoveries for the separate metals are also greater in Table A than in Table B.

15 In assaying the product, however, we have a substantially lower concentrates in Table A; 32.7 ounces of silver in the concentration of Table A compared with 43.4 ounces in Table B, and 5.05 ounces of silver in the tails of Table A compared with 6.98 ounces in Table B.

20 With the same ore, treated by my present method over a period of eight days and approximately 600 tons, the results were in accordance with Table C.

Table C

| 30                   | % Weight | Assay   |      |      |        | Recoveries—per cent |       |       |       |
|----------------------|----------|---------|------|------|--------|---------------------|-------|-------|-------|
|                      |          | Ag ozs. | Pb % | Fe % | Ins. % | Ag                  | Pb    | Fe    | Ins.  |
| Heads.....           | 100.0    | 22.6    | 18.8 | —    | 50.9   | 100.0               | 100.0 | 100.0 | 100.0 |
| Concentrates.....    | 55.8     | 36.9    | 32.3 | 9.5  | 28.2   | 91.2                | 96.1  | —     | 30.8  |
| Oxide Cl. tails..... | 8.9      | 8.6     | 4.7  | 9.9  | 67.5   | 3.4                 | 2.2   | —     | 11.8  |
| Final tails.....     | 35.3     | 3.5     | 0.89 | —    | 82.6   | 5.4                 | 1.7   | —     | 57.4  |

40 Table C shows the improvement in concentration ratio compared with Table B without sacrificing recoveries of either silver or lead values.

45 This removal of refractory values from a flotation circuit can be applied to the treatment of ores other than those cited, and I do not wish to limit my invention to those ores. For instance, in the treatment of some copper ores containing sulphide and oxide copper minerals, some oxide copper mineral would act as the cited silver minerals, in 50 which case the middling containing the refractory copper mineral would be removed from the circuit and treated separately as indicated.

55 Various other modifications may be made by those skilled in the art without departure from the invention as defined in the following claims.

1. In the concentrating by froth flotation of mixed oxide-sulphide lead-silver ores, the 60 method which consists in taking off sulphide concentrates, subjecting them to a cleaner and returning the tails to the head of the circuit, taking off oxide concentrates, subjecting them to a cleaner and passing the tails to the head of the oxide circuit and taking off

a middlings concentrate and diverting it from the circuit for further treatment.

2. In the concentrating by froth flotation of mixed oxide-sulphide lead-silver ores, the method which consists in taking off sulphide 70 concentrates, subjecting them to a cleaner and returning the tails to the head of the circuit, taking off oxide concentrates, subjecting them to a cleaner and passing the tails to the head of the oxide circuit and taking off a middlings concentrate, cleaning it and treating the cleaner concentrates and tails outside of the froth floatation circuit to recover their values.

75 In witness whereof, I have hereunto signed my name.

ALBERT W. HAHN.

85

90

95

100

105

110

115

120

125

130